

1

2,824,062

**METAL SALTS OF PHOSPHORUS PENTASULFIDE-OLEFIN REACTION PRODUCTS**

Lyle A. Hamilton, Pitman, Phillip S. Landis, Mickleton, and Francis M. Seger, Pitman, N. J., assignors to Socony Mobil Oil Company, Incorporated, a corporation of New York

No Drawing. Application December 30, 1953  
Serial No. 401,412

8 Claims. (Cl. 252—32.7)

This invention relates to a new class of phosphorus- and sulfur-containing metal salts and to mineral lubricating oil compositions containing the same.

It is well known to those familiar with the art that mineral oil products refined for their various uses are in and of themselves usually deficient in one or more respects so that their practical utility is limited even in the particular field for which they have been refined. For example, mineral oil fractions refined for use as lubricants have a tendency to oxidize under conditions of use with the formation of sludge or acidic oxidation products. These acidic oxidation products exert a corrosive action on the metal parts being lubricated, particularly the metal bearings, such as cadmium-silver alloy bearings, utilized in modern internal combustion engines. In order to prevent the formation of such products and thereby extend the useful life of the oil, it has become the practice to blend with the oil a chemical ingredient which will have the effect of inhibiting the oxidation of the oil. Such ingredients are known as oxidation inhibitors or anti-oxidants.

It is also well known that lubricating oils when utilized in internal combustion engines tend to form carbonaceous deposits which fill the slots in the oil rings causing the rings to stick and thereby materially reducing the efficiency of the engine. Chemical ingredients have also been developed which when added to an engine oil have the ability to reduce this tendency of the oil to form deposits which interfere with the function of the piston rings. These addition agents are known as detergents.

In the manufacture of lubricating oil additives particularly anti-oxidants, it is a well known practice to react hydrocarbon materials with phosphorus sulfides to produce acidic, phosphorus- and sulfur-containing reaction products which are then neutralized with basic metal salts to produce metal salt additives. Olefinic hydrocarbons of various types have been used in such manufacture. For example, mixed olefin fractions produced by the cracking of petroleum hydrocarbon materials, such as lubricating oils and waxes, have been used for this purpose. Such olefins when reacted with phosphorus pentasulfide, for example, and converted to metal salts provide highly effective anti-oxidants for lubricating oils. These salts, however, are characteristically not satisfactory as detergents. Therefore, in order to provide lubricating oils having good detergent as well as anti-oxidant character, it has been necessary to incorporate therein a separate detergent additive along with an anti-oxidant salt of this type.

We have now found, however, that olefin-phosphorus sulfide product metal salts which exhibit not only high anti-oxidant ability but which are also superior detergents for lubricating oils can be prepared by utilizing in the preparation thereof a novel type of olefinic material, viz., a mixed olefinic fraction having a continuous boiling range between about 500° F. and 1000° F. and which is produced by liquid-phase cracking, at temperatures of from about 700° F. to about 850° F., of a petrodatum

2

filtrate consisting of from about 70 to about 90 weight percent of microcrystalline wax and from about 10% to about 30% of petroleum lubricating oil, such petrodatum filtrate having a specific gravity of between about 0.87 and about 0.88 and not more than about 20 weight percent thereof boiling below about 900° F.

As far as we are aware, the particular olefinic fractions thus produced have not been known heretofore and, accordingly, they are believed to be new compositions of matter. Likewise, metal salts of the phosphorus pentasulfide reaction products of these olefins are considered to be new and different from any analogous salts known heretofore.

We have found that olefinic fractions derived from the cracking of other petroleum stocks, such as waxes and oils as shown in the prior art, after conversion to equivalent phosphorus pentasulfide metal salts, are definitely inferior as lubricating oil detergents to the metal salts contemplated herein.

15 It is, therefore, an object of this invention to provide a new specific class of olefinic materials. It is a further object to provide a new class of metal salts of reaction products of these olefinic materials with phosphorus pentasulfide. It is also an object of this invention to provide oil compositions containing the said metal salts, which compositions exhibit high detergency as well as antioxidant ability. Other and further objects of the invention will be apparent from the following description thereof.

20 The olefins contemplated herein are believed to be naphthenic in type, as it has been found that olefins of the straight-chained type derived from the cracking of predominantly straight chain paraffins, such as paraffin wax, provide inferior reaction products. Also, olefins derived from the cracking of lubricating oils of paraffinic or aromatic character are clearly inferior.

25 The petrodatum filtrate contemplated by this invention is a non-aromatic material separated in the processing of cerese wax. Two typical petrodatum filtrates utilized herein had the analytical data given in Table I. For purpose of comparison, similar data for other hydrocarbon stocks employed in the development of this invention are also listed in the table. It will be noted that the petrodatum filtrates had specific gravities of between 0.87 and 0.88, whereas other stocks, all of which proved to be unsatisfactory, where either paraffinic and had a lower gravity or were aromatic and had a higher gravity. Also, the petrodatum filtrates had boiling ranges generally of from 600° F. to 1200° F., not more than 20% thereof boiling below about 900° F. The exact structure or 30 structures present in the petrodatum filtrates which make them suitable for use in this invention are not known, although, as aforesaid, it is believed from their physical properties that a high naphthene content may account for the enhanced detergency character of the phosphorus pentasulfide metal salt reaction products thereof.

35 The cracking of the petrodatum filtrate may be carried out in a variety of ways. However, it is preferred to use a liquid-phase operation at temperatures of from 40 about 700° F. to about 800° F. A high yield of cracked distillate boiling above 500° F. is obtained when the thermal cracking operation is performed at the aforesaid temperature level under reduced pressures, i. e., about 100 mm. (absolute). Generally, the lowered pressures are utilized in conjunction with temperatures in the lower end of the aforementioned temperature range. Table II shows the olefinic fractions obtained from a number of cracking runs along with analytical data therefor. It will be noted that the fractions from petrodatum filtrate have analytical data somewhat similar, except for specific gravity, to olefinic fractions obtained from the cracking under similar conditions of other petroleum hy-

drocarbon stocks, viz., (1) "Vacwax 40" stock, which is a mixture of paraffin wax and microcrystalline wax, predominantly paraffin wax, (2) "Atlas Cylinder" stock, a heavy Mid-Continent lubricating oil vacuum distillate, (3) "345½" stock, a solvent-refined paraffin oil and (4) "307" stock, a solvent-refined Mid-Continent lubricating oil. Yet, there is a decided difference in value as detergents when these olefinic materials are converted first to the phosphorus pentasulfide reaction products and then to metal salts.

The metal salts in all cases were prepared by first reacting the cracked olefin material with from about 5 to about 30 weight percent of phosphorus pentasulfide, at a moderately elevated temperature, i. e., from about 140° C. to about 160° C., for a period of from about 1 to about 5 hours, although temperatures as low as 100° C. and longer reaction times up to, say, 10 hours or more may also be used. The reaction product was filtered in all cases to remove any unreacted phosphorus pentasulfide and then hydrolyzed with a small amount, about 5% by weight, of water and neutralized with a basically reacting inorganic metal salt, such as a metal oxide or hydroxide.

To illustrate in detail the manner of preparation of the metal salt products contemplated herein, the following specific examples are given.

#### EXAMPLE I

A 500-gram portion of olefin Cut 6 (run No. D10181, Table II) and 100 grams of  $P_2S_5$  were heated with stirring at 150–160° C. for 3 hours. The crude product was filtered with suction through paper giving 580 grams of a viscous oil. To this material in a liter flask there was added 50 grams of zinc oxide and 25 grams of water. The flask contents were heated rapidly with stirring to 150° C. and held there for 2 hours, while 13 ml. of water was collected in a side arm takeoff trap. The reaction product was filtered with suction through paper and gave 575 grams of a viscous oil. This material contained 3.34% zinc, 4.15% phosphorus and 7.78% sulfur.

#### EXAMPLE II

A 2908-gram portion of olefin bottoms from visbroken petrolatum filtrate (run No. T-850, Table II) and 222 grams of  $P_2S_5$  were stirred together at 150–160° C. for 4 hours. The resulting solution was filtered free of sludge and unreacted  $P_2S_5$ , giving 3090 grams of intermediate reaction product. A 1000-gram portion of this reaction product, 500 ml. of toluene and 80 grams of barium hydroxide octahydrate were stirred together in a 3-liter flask fitted with a stirrer, thermometer and water take-off trap. The flask contents were heated slowly to 130° C., taking off a total of 39 ml. of water after 2 hours at this temperature. The crude reaction product was filtered with difficulty and, after topping free of toluene under vacuum, gave 961 grams of viscous dark-colored material. This product contained 2.96% barium, 1.67% phosphorus and 3.27% sulfur.

#### EXAMPLE III

A 3000-gram portion of olefin bottoms from the distillation of cracked petrolatum filtrate (run No. D10474, Table II) and 580 grams of  $P_2S_5$  were stirred together at 145–148° C. for 3 hours in a 10-liter flask under nitrogen. The product was cooled to 90° C. and 150 ml. of water added dropwise in the course of one hour. The temperature was then raised to 150° C. taking off unreacted water in a takeoff device and held at this temperature for 3 hours. The product was filtered hot through "Hyflo" (a diatomaceous earth filter aid) using suction. To a 1775-gram portion of this intermediate there was added 81 grams of zinc oxide and the reactants stirred at 150° C. for 3 hours. The product was filtered

75 with difficulty through "Hyflo," giving 1801 grams of product. This product contained 3.10% zinc, 4.29% phosphorus and 4.97% sulfur.

A number of other metal salt products, all prepared in a manner similar to that shown in the foregoing examples, are listed in Table III.

#### Evaluation of products

10 The evaluation of the products of this invention, as detergents as well as inhibitors of bearing corrosion, was carried out by means of the Lauson D-4A engine test. This test rates piston cleanliness as well as bearing corrosion. The engine is inspected for cleanliness of the rings, ring grooves and piston skirt. Cleanliness ratings are made, based on a scale of from 100 to 0, a rating of 100 signifying a perfectly clean engine and a rating of 0 representing the worst possible deposit condition. The engine is perfectly clean at the start of each test and the copper-lead bearing of the engine is accurately weighed before and after the test run and the loss in weight thereof is recorded. The test involves operation of the single cylinder, 4-cycle, liquid-cooled gasoline engine for 100 hours under the following conditions:

|                          |          |      |
|--------------------------|----------|------|
| Oil temperature          | °F       | 270  |
| Jacket temperature       | °F       | 212  |
| Speed                    | R. P. M. | 1825 |
| ½ throttle               |          |      |
| 13.0–1 air-fuel ratio    |          |      |
| Oil added every 20 hours |          |      |

The fuel used in all tests was a blended gasoline consisting of 40% thermal, 30% catalytically cracked and 30% straight run plus 2.5 cc. TEL/gal.

35 Table III shows the results of tests conducted on a number of oil blends containing metal salt products prepared from olefinic fractions produced in the cracking of petrolatum filtrate as contemplated herein. Also, for comparison, it also shows results obtained with oil blends of products produced from olefinic fractions obtained by cracking a number of other hydrocarbon oils and waxes. The base oil used in all of the test blends was an S. A. E. 20 grade, solvent-refined Pennsylvania oil having a kinematic viscosity of 63 centistokes at 100° F. It will be seen that the oil blends of the products contemplated herein gave consistently good detergency (cleanliness) ratings, i. e., from 73 upwards to as high as 85, while that of all the other products were relatively poor. It is believed that these data clearly demonstrate that the metal salt products produced from the cracked petrolatum filtrate (microcrystalline wax-oil mixture) as herein contemplated, provide unexpectedly high detergency activity in lubricating oils over the metal salt products prepared from other olefinic stocks.

40 As has been stated hereinbefore, the cracking of the petrolatum filtrate may be carried out in any suitable manner to give olefinic fractions satisfactory for use in this invention. However, we have found that the consistently best results are obtained by the use of thermal, liquid-phase cracking under either atmospheric or reduced pressures as low as about 50 mm. (absolute pressure) or lower, at temperatures of about 700° F. to about 850° F., the lower temperatures within this range being preferred where lowered pressures are employed. Also, it is preferable to use the highest boiling olefinic fractions, i. e., those having continuous boiling ranges above about 500° F. and preferably within the limits of from about 500° F. to about 1000° F., in order to provide oil solubility in the reaction products. However, the use of small amounts, i. e., from about 10% to about 20%, of olefins having a 400° F. to 500° F. boiling range along with higher boiling olefins will provide highly satisfactory products.

45 50 55 60 65 70 75 76 The metal salts contemplated herein are those of the

metals of Group II of the Mendeleeff Periodic Table, particularly the salts of barium, calcium, magnesium, strontium and zinc, with the barium salts being especially preferred.

The amount of metal salt reactant product to be utilized in the oil will range generally from about 0.5% to about 10% by weight and usually will be from about 1% to

about 5%, depending upon the particular oil to be improved and the application for which it is intended.

It is also contemplated that other additives designed to improve the oil in various respects, such as pour depressants, viscosity improvers, extreme pressure agents, etc., may also be used in the oil along with the additives herein contemplated.

TABLE I.—CHARGE STOCKS FOR LIQUID-PHASE CRACKING

| Identification           | Petrolatum Filtrate "A" | Petrolatum Filtrate "B" | Vacwax 40 | 345½ P. D. Raffinate | 345½ Furfural Raffinate | 307 Stock |
|--------------------------|-------------------------|-------------------------|-----------|----------------------|-------------------------|-----------|
| Specific Gravity         | 0.8772                  | 0.8772                  | 0.8413    | 0.9303               | 0.8916                  | 0.8911    |
| Viscosity, cs. @ 210° F. | 25.85                   | 20.58                   | 6.58      | 30.84                | 18.97                   | 17.65     |
| Vacuum Assay:            |                         |                         |           |                      |                         |           |
| IBP (° F.)               | 720                     | 620                     | 725       | 745                  | 635                     | 750       |
| 10.                      | 955                     | 860                     | 870       | 920                  | 790                     | 800       |
| 20.                      | 994                     | 915                     | 890       | 935                  | 855                     | 830       |
| 30.                      | 1,050                   | 960                     | 900       | 970                  | 940                     | 840       |
| 40.                      | 1,080                   | 1,005                   | 920       | 992                  | 1,005                   | 865       |
| 50.                      | 1,095                   | 1,050                   | 930       | 1,020                | 1,040                   | 910       |
| 60.                      | 1,130                   | 1,100                   | 935       | 1,045                | 1,075                   | 960       |
| 70.                      |                         | 1,140                   | 940       | 1,090                | 1,095                   | 1,030     |
| 80.                      |                         |                         | 950       | 1,100                |                         | 1,100     |
| 90.                      |                         |                         | 960       |                      |                         | 1,150     |
| 95.                      |                         |                         | 1,000     |                      |                         |           |
| Molecular Weight         | 710                     | 660                     | 480       | 580                  | 590                     | 585       |
| Bromine Number           | 1.1                     | 3.6                     | 0.7       | 10.5                 | 3.7                     | 3.2       |
| Olefin Content, Percent  | 5                       | 15                      | 2         |                      | 14                      | 12        |

TABLE II.—OLEFINIC FRACTIONS FROM CRACKED STOCKS<sup>1</sup>

| Cracking Charge                           | Fraction Utilized | Liquid Recovery, Wt. Percent | Distillation Range, ° F. | Specific Gravity | Br. No. | Mol. Wt. | Olefin Content, Percent |
|-------------------------------------------|-------------------|------------------------------|--------------------------|------------------|---------|----------|-------------------------|
| Petrolatum Filtrate                       |                   |                              |                          |                  |         |          |                         |
| T850, Bottoms                             | 90                | 510-1,100                    | 0.8660                   | 11.2             | 570     | 40       |                         |
| D3902, Bottoms                            | 35                | >700                         | 0.8866                   | 21.5             | 600     | 84       |                         |
| D211, Bottoms                             | 78                |                              |                          |                  |         |          |                         |
| D10181, Cut 5                             | 12                | 517-604                      | 0.8270                   | 46.4             | 242     | 70       |                         |
| Cut 6                                     | 19                | 602-636                      | 0.8358                   | 32.9             | 308     | 63       |                         |
| Bottoms                                   | 48                | 672-894                      | 0.8565                   | 17.6             | 400     | 44       |                         |
| D10474, Bottoms                           | 78                | 510-953                      | 0.8607                   | 26.1             | 380     | 62       |                         |
| D10178, Cut 4                             | 18                | 396-498                      | 0.7870                   | 48.3             | 190     | 57       |                         |
| Cut 5                                     | 21                | 515-590                      | 0.8008                   | 34.6             | 238     | 51       |                         |
| Bottoms                                   | 26                | 565-751                      | 0.8165                   | 15.2             | 300     | 29       |                         |
| Vacwax 40                                 | do                | 47                           |                          | 0.9478           | 23.6    | 440      | 65                      |
| 345½ Stock Propane Deasphalting Raffinate | do                | 49                           |                          | 0.8950           | 17.5    | 470      | 51                      |
| 345½ Stock Furfural Raffinate             | do                | 12                           | 615-782                  | 0.8927           | 23.2    | 325      | 47                      |
| 307 Stock Propane Deasphalting Raffinate  | do                | 34                           | 630-840                  | 0.8973           | 24.6    | 330      | 51                      |
| Atlas Cylinder Stock                      |                   |                              |                          |                  |         |          |                         |

<sup>1</sup> All cracking runs except T850 and D3902 were by batch liquid-phase operation at 700-750° F. The T850 run was made by cracking in a coil under vis-breaking conditions. Run D3902 was vapor-phase cracking at 1050° F.

TABLE III.—ADDITIVES PREPARED FROM CRACKED STOCKS

| Source                                    | Fraction                       | Additive Preparation and Analyses |            |            | Lauson D-4-A Evaluation      |                           |                    |                     |
|-------------------------------------------|--------------------------------|-----------------------------------|------------|------------|------------------------------|---------------------------|--------------------|---------------------|
|                                           |                                | Metal, Percent                    | P, Percent | S, Percent | Percent Additive in Test Oil | Percent Metal in Test Oil | Cleanliness Rating | ½ Brg. Wt. Loss, g. |
| Petrolatum Filtrate                       | T-850, Bottoms                 | None                              | 1.7        | 3.6        | None                         | None                      | 52                 | 0.280               |
| 345½ Stock Propane Deasphalting Raffinate | Bottoms                        | Barium, 5.3                       |            |            | 5.9                          | 0.2 Ba                    | 57                 | 0.002               |
| 307 Stock Propane Deasphalting Raffinate  | D-209, Bottoms                 | Barium, 1.45                      | 1.81       | 3.86       | 13.8                         | 0.2 Ba                    | 47                 | 0.006               |
| Atlas Cylinder Stock                      | D-213, Bottoms                 | Sodium, 1.06                      | 0.87       | 1.85       | 2.9                          | 0.034 Na <sup>2</sup>     | 62                 | 0.004               |
| Vacwax 40                                 | D-10178, Cuts 4, 5 and Bottoms | Zinc, 2.9                         | 4.86       | 7.47       | 2.0                          | 0.058 Zn                  | 61                 | 0.010               |
| Petrolatum Filtrate                       | T-850, Bottoms                 | Barium, 2.96                      | 1.67       | 3.27       | 3.4                          | 0.1 Ba                    | 85                 | 0.003               |
| Do                                        | do                             | Barium, 1.69                      | 1.67       | 3.56       | 5.9                          | 0.1 Ba                    | 81                 | 0.003               |
| Do                                        | T-850, Bottoms <sup>1</sup>    | Barium, 2.64                      | 1.44       | 2.92       | 3.8                          | 0.1 Ba                    | 69                 |                     |
| Do                                        | D-3902, Bottoms                | Barium, 5.62                      |            |            | 7.6                          | 0.2 Ba                    | 77                 |                     |
| Do                                        | do                             | Barium, 4.2                       | 1.73       | 2.94       | 3.6                          | 0.2 Ba                    | 79                 | 0.023               |
| Do                                        | D-211, Bottoms                 | Barium, 3.0                       | 1.89       | 3.57       | 4.8                          | 0.2 Ba                    | 73                 | 0.003               |
| Do                                        | do                             | Calcium, 1.42                     | 2.05       | 3.09       | 6.7                          | 0.2 Ba                    | 75                 | 0.009               |
| Do                                        | do                             | Barium, 5.1                       | 1.94       | 4.06       | 4.1                          | 0.058 Ca <sup>2</sup>     | 74                 | 0.002               |
| Do                                        | do                             | Barium, 1.8                       | 1.48       | 3.04       | 3.9                          | 0.2 Ba                    | 73                 | 0.002               |
| Do                                        | D-211, Bottoms <sup>1</sup>    | Barium, 3.6                       | 1.81       | 3.54       | 5.6                          | 0.2 Ba                    | 76                 | 0.002               |
| Do                                        | D-211, Bottoms                 | Zinc, 2.1                         |            |            | 4.5                          | 0.095 Zn <sup>2</sup>     | 78                 | 0.006               |
| Do                                        | D-10181, Cut 6                 | Zinc, 3.34                        | 4.15       | 7.78       | 2.0                          | 0.068 Zn <sup>2</sup>     | 80                 | 0.001               |
| Do                                        | do                             | Zinc, 2.82                        |            |            | 2.0                          | 0.056 Zn                  | 75                 | 0.002               |
| Do                                        | D-10181, Cuts 5, 6 and Bottoms | Barium, 3.7                       | 4.19       | 3.99       | 2.0                          | 0.08 Ba                   | 73                 | 0.018               |
| Do                                        | do                             | Barium, 3.4                       |            |            | 5.9                          | 0.2 Ba                    | 73                 | 0.051               |
| Do                                        | D-10474, Bottoms               | Zinc, 2.87                        | 4.16       | 5.40       | 2.0                          | 0.058 Zn <sup>2</sup>     | 80                 | 0.007               |
| Do                                        | do                             | Zinc, 2.98                        | 4.06       | 5.40       | 1.0                          | 0.030 Zn                  | 72                 | 0.007               |
| Do                                        | do                             | Zinc, 2.98                        | 4.06       | 5.40       | 2.0                          | 0.059 Zn                  | 75                 | 0.007               |
| Do                                        | do                             | Zinc, 3.10                        | 4.06       | 5.40       | 4.0                          | 0.118 Zn                  | 81                 | 0.008               |
| Do                                        | do                             | Zinc, 3.10                        | 4.29       | 4.97       | 8.0                          | 0.236 Zn                  | 81                 | 0.010               |
| Do                                        | do                             | Zinc, 3.10                        | 4.29       | 4.97       | 2.0                          | 0.060 Zn                  | 85                 | 0.007               |

<sup>1</sup> Percolation of olefinic material before P<sub>2</sub>S<sub>5</sub> reaction reduced color and specific gravity with slight reduction in bromine number.

<sup>2</sup> 0.2% barium equivalent to 0.095% zinc; 0.058% calcium; 0.067% sodium.

Having now fully described the invention, what is claimed as new and patentable is:

1. As a new composition of matter, a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with a basically reacting metal salt of a metal selected from group II of the periodic table, to form a metal salt thereof.

2. As a new composition of matter, a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with barium hydroxide to form a barium salt thereof.

3. As a new composition of matter, a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with calcium hydroxide to form a calcium salt thereof.

4. As a new composition of matter, a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with zinc hydroxide to form a zinc salt thereof.

5. A mineral lubricating oil containing from about 0.5 to about 10 percent by weight of a metal-, phosphorus- and sulfur-containing product produced by the steps of (1) reacting (A) an olefinic hydrocarbon material having a continuous boiling range of from about 500° F. to about

1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil; (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with a basically reacting metal salt of a metal selected from group II of the periodic table, to form a metal salt thereof.

15 6. A mineral lubricating oil containing from about 0.5 to about 10 percent by weight of a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with barium hydroxide to form a barium salt thereof.

20 7. A mineral lubricating oil containing from about 0.5 to about 10 percent by weight of a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with calcium hydroxide to form a calcium salt thereof.

25 8. A mineral lubricating oil containing from about 0.5 to about 10 percent by weight of a metal-, phosphorus- and sulfur-containing product produced by the steps of (1) reacting (A) an olefinic hydrocarbon material having a continuous boiling range of from about 500° F. to about 1000° F., produced by the liquid-phase thermal cracking at a temperature of from about 700° F. to about 850° F., of a petrolatum filtrate characterized as follows: (a) consisting of from about 70 to about 90 weight percent of microcrystalline wax and the remainder lubricating oil, (b) having a specific gravity of from about 0.87 to about 0.88 and (c) not more than 20% thereof boiling below about 900° F. with (B) from about 5 to about 30 weight percent of phosphorus pentasulfide at a temperature of from about 100° C. to about 160° C. to form an acidic, phosphorus- and sulfur-containing product and (2) reacting the product of step 1 with zinc hydroxide to form a zinc salt thereof.

References Cited in the file of this patent

| UNITED STATES PATENTS |                 |               |
|-----------------------|-----------------|---------------|
| 2,316,088             | Loane et al.    | Apr. 6, 1943  |
| 2,476,812             | Buckmann et al. | July 19, 1949 |
| 2,507,731             | Mixon et al.    | May 16, 1950  |
| 2,673,831             | Hughes          | Mar. 30, 1954 |